

March 3, 1936.

W. B. WESCOTT

2,032,779

FLEXIBLE COMPOSITE PLANOGRAPHIC PLATE

Filed Jan. 26, 1934



*Inventor  
William B. Wescott  
of Roberts, Culver & Wescott  
this 26th day of January  
1934.*

## UNITED STATES PATENT OFFICE

2,032,779

## FLEXIBLE COMPOSITE PLANOGRAPHIC PLATE

William B. Wescott, Dover, Mass., assignor to  
Multigraph Company, Wilmington, Del., a corporation of Delaware

Application January 26, 1934, Serial No. 708,398

10 Claims. (Cl. 101—401)

This invention relates to an improvement in a planographic plate, and more particularly to a flexible composite planographic plate which comprises a flexible cellulosic base surfaced with closely packed discrete metallic particles firmly adherent thereto.

The planographic plates of this invention, while useful for planographic printing generally, have particular utility in connection with printing images produced thereon by direct typewriting. The ordinary sheet-metal planographic plate is not adapted to take a printing image directly from a typewriter.

I am aware that thin paper-backed metal foil has heretofore been proposed and used for the production of a printing image by direct typewriting; but, if the foil is thin enough to afford the requisite flexibility, it is disadvantageously embossed by the action of graining marbles; and, if thick enough to prevent embossing thereby, it will not readily conform to the platen roll of, nor take a clean impression in, the usual typewriter. I am also aware that it has heretofore been proposed to overcome the difficulties inherent in sheet-metal plates by spraying molten metal on a flexible non-metallic backing; but, the surface, of the sprayed particles, becomes oxidized during the spraying operation and hence the facings obtained therefrom are disadvantageously permeated with oxide which cannot be eliminated by the customary treatment for the removal of surface oxide from planographic plates; moreover the metal facings so obtained have little tensile strength, and disadvantageously crack when bent around the typewriter platen and, what is more important, about the form roll of the press.

One object of this invention is to provide a planographic plate adapted to take a clean image by direct typewriting in a usual typewriter. Another object is to provide a composite plate of high flexibility which may be made to conform to typewriter platens of small radius without detriment. Still another object is to provide a composite plate having a metallized printing surface, comprising closely packed discrete particles of metal, preferably zinc, which, while firmly adherent to the supporting base, are so exposed as to be chemically reactive with image-forming inks and ink-repellent solutions. Other objects and advantages of the invention will become apparent as its description proceeds.

The art of planographic printing depends upon the immiscibility of oil and water and the ability of water to displace or repel ink from a

surface more readily wet by water than by oils. In direct planography a greasy image is produced directly on a metal surface by any convenient means. The effective retention of this image by the metal, under printing conditions, depends upon a chemical reaction between constituents of the greasy image-forming material and the metal. The preservation of the non-printing areas of the plate during the inking and printing operations also depends upon a chemical reaction between the metal and constituents of a dampening solution applied thereto, whereby the metal of the non-printing areas is rendered preferentially water-receptive, or lyophilic. The metal constituting the printing surface of the plate, to be effective for the purpose, must therefore be so exposed as to be chemically reactive. It is generally considered essential and it is certainly highly desirable, that the printing surface be slightly rough or "grained".

For a clear understanding of the present invention, it is necessary to consider the role played by the "grain" of a planographic plate. A film of water on a smooth plate has two surfaces of equal extent; whereas on a grained plate the extent of the water-air surface is much less than is the extent of the water-metal surface. If the surface tension of the aqueous fluid and the wettability of the metal thereby are respectively the same in both cases, it is obvious that a film of the aqueous fluid will offer a greater resistance to displacement from the grained surface than from the smooth surface, because the ratio of water-metal surface to water-air surface is greater in the former than in the latter, while the ratio of surface tension to metal-wettability remains the same in both cases. It is, however, also obvious that any attritional wear of the grained surface must occur at the apices of the grain; and it is common experience that, unless continuously treated during printing to maintain these apices in a lyophilic condition, they soon lose their preferential water-wettability, pick up ink, and produce a speckled effect on the whites of the print. From this observation it has been generally held that, to obtain clean prints from a planographic plate, the entire non-printing area thereof must be rendered and maintained in a preferentially water-wettable condition throughout the printing operation.

The present invention has its genesis in the discovery that the non-printing area of a grained planographic plate need not be rendered lyophilic throughout its entire extent, in order to

effectively prevent contamination thereof by the printing ink, provided the residual ink-receptive portions thereof be minute and be restricted to the valleys formed by and between adjacent grain prominences.

The planographic plate of this invention comprises essentially a cellulosic base surfaced with a coextensive layer of firmly adherent, closely packed discrete particles of metal, preferably zinc. 10 For a clear understanding of the invention and for visualization of the disposition of these metallic particles to each other and to the supporting base, reference is had to the drawing in which

15 Fig. 1 is a somewhat schematic view in plan, of a portion of a plate of this invention, representing in line drawing the general configuration of the particles as seen at a magnification of about 500 diameters; and

20 Fig. 2 is an enlarged cross section thereof.

In the embodiment of the invention illustrated in the drawing, metal particles A and B are partially embedded in a bonding matrix C, which may be either the substance of the cellulosic base D or a layer of a suitable adhesive.

In any event, close packing of the metal particles is desired in order that the area of the exposed matrix C be at a minimum, and for this purpose it has been found desirable, but not 30 always necessary, to use particles of two widely variant sizes, as indicated by the large particles A which determine the "graininess" of the plate and by the small particles B which serve to reduce the uncovered areas therebetween. Where 35 a "grain" of very fine texture is desired, a single screen-sized (or, preferably air-separated) particle of very small mean dimensions may be used alone; but where a relatively coarse "graininess" is wanted, there is advantage in reducing 40 the interstices between large particles by affixing therein particles of a lower order of size, as B in Figs. 1 and 2.

While the process of producing the plates of this invention is not considered as being a part 45 of the present disclosure, it is, nevertheless, necessary, for clarity of presentation and understanding of the invention, to make reference to process steps.

When particles of two screen-sizes are used, it 50 will be found desirable to apply, as in the usual bronzing machine, the larger sized particle first and to apply the smaller sized particle as a separate and subsequent operation, albeit while the bonding agent is still in a tacky condition; for 55 it has been observed that a more consistently uniform texture and better coverage may be so obtained than can be had when particles of variant sizes are mixed and applied in one operation.

60 As stated, the bonding matrix C may be either the substance of the cellulosic base or it may be a layer of adhesive. Any bonding agent which adhesively wets the metal particles, which is not thermoplastic at ordinary temperatures, and which, in the dry and hardened state, is flexible and substantially inert in the contacting presence of aqueous solutions and siccative oils, may be used for the purposes of this invention. Synthetic resinous condensation products, which, 65 after final condensation, retain a high degree of flexibility, are useful for the purposes of this invention; particularly in that, as no solvent is required, they remain of constant tackiness until 70 subjected to the final condensation, and hence 75

are well adapted to the sequential application of metal particles of different size.

Any suitable cellulosic base may be used. The base material may be solid, as sheeted cellulose acetate or nitrate, or it may be open textured as paper or cloth. Paper tends to split along its lamina under the rolling action of the inking and transfer mechanism in a rotary offset press; and, therefore, requires in general to be unified as by impregnation with a bonding agent. For 10 the purposes of this invention it has been found convenient and satisfactory to effect a substantial unification of the constituent fibers of the paper by partial or complete impregnation of the interfiber space by the flexible bonding agent, which also serves to hold the metal particles at 15 the surface.

In general it is enough that the bonding agent penetrate somewhat more than half way through the paper base. Complete impregnation through 20 to the back of the paper is not only not essential to the satisfactory functioning of the product, but it involves unjustified process complications.

For reason of economy there is sometimes advantage in metallizing both surfaces of a flexible 25 cellulosic base. When such a double surfaced planographic plate is produced on a paper base, according to this invention, substantially complete impregnation of the pores of the paper is, if not essential, at least highly desirable. Such 30 a substantially complete impregnation is obtained by the sequential treatment of the two surfaces, thereby avoiding the mentioned process complications.

When a cloth base is used, it is enough that 35 the bonding agent so penetrate the interstices of the superficial fibers as to obtain good anchorage, as the cloth may be said to be inherently and structurally unified in the sense in which that expression is used herein.

40 Particles of metal of widely variant shapes may be used for the surfacing of the plates of this invention. Thus pellets previously derived from sprayed metal, or the more irregular particles derived from grinding, may be used in the conventional bronzing machines. Metal flakes, as derived from tumbling extremely thin metal foil, may be used; but due to the fact that they are thin, and in consequence tend to lie parallel to the plane of the base, they are not ordinarily 45 so effective to hold the dampening fluid in their interstices as are the thicker pellets or irregular particles. If, however, they are so oriented, as in an electrostatic field, as to first contact the adhesive at an edge rather than flat, they may 50 be subsequently laid down in an overlapping arrangement, somewhat similar to that of fish scales, by a unidirectional brushing operation. Such a "fish scale" disposition of metallic flakes is effective to greatly reduce the uncovered areas. 55 It should be noted that where metallic flakes have been laid down in overlapping arrangement, the resulting plate must, for best results, be so oriented on the form roll of the press that on 60 rotation thereof the fixed edge of the flakes are 65 to the fore; that is, the direction in the press must be the same as that which produced the overlap.

To the extent that any areas of exposed bonding agent persist, and whether the particles be 70 flakes or granular, the same considerations obtain. These considerations are that the largest interstitial area, between any adjacent particles, should not appreciably exceed the mean cross-sectional area of the largest of the particles con- 75

stituting the coating; and that the mean interstitial area between adjacent particles should be substantially less than the average mean cross-sectional area of the particles. Absolute limits of permissible uncovered areas cannot be given because their innocuousness does not depend upon the smallness of area alone, but also depends upon the height of the particles bounding the area, and also upon the viscosity and surface tension of the dampening fluid used on the plate.

The particle size may be varied over fairly wide limits as the character of the ink to be used, the nature of the work to be printed, and the viscosity and surface tension of the dampening fluid may dictate. But, in general, it has been found that the largest useful particles are of the order of 0.01 mm. in mean diameter, and that, for the usual run of printing and particularly when an effective dampening solution (such as that disclosed in my copending application Serial No. 689,285 which has matured into Patent No. 2,003,268, May 28, 1935) is used, best results are obtained when the particles, imparting the graininess and effecting most of the coverage, are closely sized to a mean diameter of about 7.5 microns and the smaller particles, applied to reduce the uncovered area, are 0.5 to 1.5 microns in mean diameter.

While zinc is the metal preferred for the purposes of this invention, other metals, such as aluminum, for instance, and alloys of these and/or other metals such as magnesium and cadmium may be used.

From the standpoint of economy, an unsized paper is preferred as the cellulosic base of the plates of this invention. However, sheet cellulose acetate or nitrate, woven fabric, or other sheet cellulosic material, may be used.

I sometimes find it desirable to "counteretch", or sensitize to the fatty acids of grease, the metal particles before effecting their attachment to the base material, and thereby obviate the necessity for the performance of this operation by the user of the plate. Because all the metals, useful for the purposes of this invention, oxidize more or less rapidly, and because the presence of oxide is detrimental to the formation of a persistently retentive image, it is not enough that the counteretch should remove the oxide, but it should also replace it with a basic product, as basic aluminum sulphate, for instance.

As stated, there is advantage and economy in providing a plate with both surfaces prepared for planographic use. A method of protecting one side of a double-faced plate comprises essentially rolling into contact with the to-be-protected side, a sheet of thin flexible material, as paper, regenerated cellulose, etc., coated with a dry, aggressively adhesive material, as crude rubber and coumarone resin or Burgundy pitch. These coatings are so well known as to need no further description here except to say that they effectively protect the underlying metallized surface from such contamination as would normally be incident to the usual manipulations of the plate in preparation for and during use.

Careful investigation of the properties of commercially available metallized papers has failed to discover any which conform to the requirements of this invention. So far as could be ascertained, the heretofore metallized papers had at least one objectionable characteristic; which is that the disposition of the metal particles, predominantly flakes, produced patches of closely packed particles with intervening uncovered

areas greatly in excess of the mean particle size.

Moreover the metal was not found to be uniformly chemically reactive, either because it was protectively coated with a practically unremovable layer of stearate derived from the usual method of producing metal flakes from foil, or because it was so embedded in the bonding agent as to be substantially covered thereby.

As stated, for the purposes of this invention the metal particles must be chemically reactive; that is, they must not be submerged in the bonding agent nor coated with water-insoluble material. Moreover, in order that the area of uncovered bonding agent may be at a minimum, it is desirable that the contact between the particles and the bonding agent be restricted to the lower portion of the former.

When the use of a very soft ink is required and the dampening fluid is incapable of preventing such ink from contacting the uncovered areas of the bonding material, it has been found possible so to modify the reactive surfaces of the metallic particles as to counteract the contaminating effect of the soft ink. This modification is obtained, in the case of zinc, by treating the reactive surfaces of the zinc particles, after the greasy image has been delineated on the plate, with a half molar solution of ammonium dihydrogen phosphate (or alternatively the sodium or potassium salt) for five to ten minutes. Microscopic inspection of so-treated zinc particles discloses the fact that their reacted surfaces are covered with fine crystalline excrescences, and that these tend substantially to fill the interstices being interlaced across the interstices between adjacent grains. The structure of the crystalline product of the reaction has not been definitely ascertained; but, for the purposes of this disclosure, it is referred to as, in the case of zinc, an insoluble zinc ammonium phosphate.

By the expression "closely packed," as used herein, is meant such a juxtaposition of the particles that the ratio of metal-covered surface to uncovered surface is substantially constant for all similar small areas, and that the mean area of the uncovered interstitial surfaces is less than the average mean cross sectional area of the particles used; and, in any event, does not exceed a mean area of 100 sq. microns.

The expression "firmly adherent", as used herein, is meant to denote such an adherence as will effectively resist the pull of a tacky ink. If the strength of the bond between base and metal particles is such that the metal particles are not extirpated when rolled up with an ink of greater tack than can be distributed by the conventional ink rolls, the particles are deemed to be firmly adherent within the meaning of that expression as herein used.

The expression "unified cellulosic base", as used herein, is meant to include a base comprising cellulose fibers cementitiously bonded to at least half the thickness of the base, as by a permeating impregnant, as well as a solid composition derived from cellulose.

The expression "discrete metal particles" as used herein, is meant to denote metallic particles which have no metallic bond with each other, even though they be in contact as may be demonstrated by electrical conductivity of a film composed of such contacting discrete metallic particles; and to specifically exclude particles which have a metallic bond, as by being fused together.

I claim:

1. A flexible planographic plate comprising a unified cellulosic base, a layer of closely packed discrete metallic particles firmly adherent thereto, and an ink receptive image applied directly to the metallic particles.
2. A flexible planographic plate comprising a unified cellulosic base, a water-insoluble bonding agent adherent to said base, a layer of closely packed discrete metallic particles firmly adherent to said bonding agent, and an ink receptive image applied directly to the metallic particles.
3. A flexible planographic plate comprising an open-textured cellulosic base, a water-insoluble bonding agent penetrating said base and coextensive with a surface thereof, a layer of closely packed discrete metallic particles coextensive with and firmly adherent thereto, and an ink receptive image applied directly to the metallic particles.
4. A flexible planographic plate comprising an open-textured cellulosic base, a water-insoluble bonding agent permeating said base, a layer of closely packed discrete metallic particles coextensive with said base and firmly adherent thereto, and an ink receptive image applied directly to the metallic particles.
5. A flexible planographic plate comprising a unified cellulosic base, a layer of discrete metallic particles firmly adherent thereto and characterized by the fact that each of said particles closely approximates a plurality of other particles, and that the mean area of the base exposed by the interstices between adjacent particles is substantially less than the average mean cross sectional area of the particles, and that the largest area so exposed between any adjacent particles is less than the mean cross sectional area of the largest of said particles, and that the mean interstitial area between adjacent particles is substantially less than the average mean cross sectional area of said particles, and an ink receptive image applied directly to the metallic particles.
6. A flexible planographic plate comprising a unified cellulosic base, a layer of discrete metallic particles firmly adherent thereto and characterized by the fact that each of said particles closely approximates a plurality of other particles, and that the mean area of the base exposed by the interstices between adjacent particles is substantially less than the average mean cross sectional area of the particles, and an ink receptive image applied directly to the metallic particles.
7. A flexible planographic plate comprising a unified cellulosic base, a layer of discrete metallic particles firmly adherent thereto and characterized by the fact that each of said particles closely approximates a plurality of other particles, and that the mean area of the base exposed by the interstices between adjacent particles is substantially less than the average mean cross sectional area of the particles, and that the largest area so exposed between any adjacent particles is less than the mean cross sectional area of the largest of said particles, and that the mean interstitial area between adjacent particles is substantially less than the average mean cross sectional area of said particles, and an ink receptive image applied directly to the metallic particles.
8. A flexible planographic plate comprising a unified cellulosic base surfaced with firmly adherent discrete particles of zinc characterized by the fact that the interstices between said particles are substantially filled by a phosphate of zinc and a metal of the alkali metal group.
9. A flexible planographic plate comprising a unified cellulosic base surfaced with firmly adherent discrete particles of zinc characterized by the fact that the interstices between said particles are substantially filled by zinc ammonium phosphate.
10. A flexible planographic plate comprising a unified cellulosic base surfaced with firmly adherent discrete particles of zinc characterized by the fact that the said particles are substantially covered by a basic metal salt.

35  
40  
WILLIAM B. WESCOTT.